

(No Model.)

J. A. HOUSE.  
Corset Stiffener.

No. 242,537.

Patented June 7, 1881.

Fig. 1.



Fig. 3.



Fig. 2.



Fig. 4.



Fig. 5.



Fig. 7.



Fig. 5.



Fig. 8.



Fig. 9.



Inventor.

J. A. House  
By his attorney  
Charles E. Minter

Attest:  
Courtney A. Corcoran  
J. C. McCleary.

# UNITED STATES PATENT OFFICE.

JAMES A. HOUSE, OF BRIDGEPORT, CONNECTICUT, ASSIGNOR TO WARNER BROTHERS, OF NEW YORK, N. Y., AND OF BRIDGEPORT, CONNECTICUT.

## CORSET-STIFFENER.

SPECIFICATION forming part of Letters Patent No. 242,537, dated June 7, 1881.

Application filed January 22, 1881. (No model.)

*To all whom it may concern:*

Be it known that I, JAMES ALFORD HOUSE, of Bridgeport, Fairfield county, Connecticut, have invented certain Improvements in the 5 Manufacture of Corset-Stiffeners, &c., of which the following is the specification.

My invention is an improvement in the construction of that class of stiffening-ribs used for imparting rigidity to corsets and bosom-pads, and composed of fibers of stiff material bound together; and my improvement consists in the mode of manufacturing such articles whereby to secure ribs or blades of any desired 10 size or shape, and in the article thus produced.

15 The improved ribs or blades are made from any stiff elastic fibers or splints, such as tam-pico fibers alone or combined with blades of horn or other material, the said fibers being collected in a bunch or bundle of the required 20 form, and then united or consolidated by means of threads combined therewith, so as to hold each blade or fiber in its position relative to the others.

Different modes of combining the threads 25 with the fibers may be employed so as to secure the desired result. One mode which I have adopted consists in first forming a continuous strip or a rib by binding in a bundle a mass of splints or fibers, *a*, by means of wrapping-threads *b*, or by metal bands, or in any 30 other manner, then combining two or more of the ribs thus made by arranging them side by side, as shown in Fig. 1, and uniting the same in such manner as to retain them firmly in juxtaposition, consolidating the whole so as to form 35 a blade in which the fibers are compacted firmly and solidly together, forming a stiff yet elastic blade, which as thus made, or as further stiffened as described hereinafter, is adapted to be 40 used as a substitute for the ordinary blades of bone or horn usually employed as stiffeners for corsets.

The binding may be effected by threads passing round or through the mass of fibers in different ways to hold them compactly together. 45 As shown in Fig. 2, some of the threads pass over and under the fibers and others pass through the mass, tying the upper and lower threads tightly down upon the faces of the 50 blade.

Instead of binding the ribs *a*, as described, before combining them, the separate unbound bundles of fiber may be brought together and united by threads, as shown in Figs. 3 and 4, the result being the same so far as concerns 55 the consolidating, condensing, or compacting of the mass of fibers in one broad flat blade.

Any desired means may be employed whereby the fibers are collected together and formed into continuous bundles or ribs *a* of unlimited 60 length, thereby utilizing short fibers, which could not otherwise be employed in the manufacture of long blades. In like manner I can form long continuous blades of combined fibers and horn strips, utilizing short thin pieces of 65 horn or other material which could not well be embodied in long blades in any other manner. Thus short strips *e e* of horn may be arranged between and combined with continuous ribs *a* of fiber, and all may be consolidated by any 70 surrounding binding, as in Figs. 5, 6, and 7; or the strips of horn may be superposed on the ribs and united thereto, as shown in Fig. 8. In any case the short horn is made the means of producing a long stiffening-blade, while 75 greater stiffness is imparted to the latter than would result from the use of fiber alone.

To facilitate the combination of the short strips *e* with the continuous ribs *a*, the horn strips may be bound together in continuous 80 lengths by wrapping-threads, as shown in Fig. 9, thus permitting all the ribs which are to be united in the blade to be manipulated in like manner, and avoiding the necessity of feeding the short strips separately. Cement may be 85 substituted for binding-threads to unite the strips *e*.

Where it is desirable or necessary to form a blade of greater stiffness or rigidity, I apply to the material, at any stage during the manufacture, a waterproofing or stiffening composition, as marine glue, japan, paint, or other suitable material, which will fill the interstices of the blade and make the same more solid and durable by securing a closer union of the fibers and 90 preventing the entrance of moisture. I do not claim this, however, as my invention. The blade may also be compacted by the application of pressure, and the further application of 95 heat is sometimes advantageous—as, for in- 100

stance, when tampico is employed, the fibers being thereby rendered stiffer and more elastic.

Any suitable apparatus may be employed for facilitating the above-described mode of manufacture, and I have used appliances which I do not here describe, as the same will constitute the subject of a separate application for Letters Patent.

I do not claim a stiffener composed of tampico fibers bound together, as this is not my invention; but

I claim—

1. The mode herein described of constructing stiffeners for corsets, the same consisting in collecting together two or more ribs of stiff elastic fibers or splints, formed substantially as described, and uniting the same to form a flat blade, substantially as set forth.

2. The improvement in the manufacture of

corset-stiffeners consisting in forming fibers of stiff elastic material into ribs and binding together the ribs by threads to form a flat blade, substantially as set forth.

3. The combination, in a corset-stiffener, of a series of fibers of stiff elastic material, such as tampico and strips of horn, substantially as set forth.

4. As a new article of manufacture, a corset-stiffener consisting of ribs of stiff elastic material united to form a flat blade, substantially as set forth.

In testimony whereof I have signed my name to this specification in the presence of two subscribing witnesses.

JAMES ALFORD HOUSE.

Witnesses:

CHARLES H. DIMOND,  
JAMES CARR.